

## UNITED STATES PATENT OFFICE

CHARLES H. WATERS, OF OLYMPIA, WASHINGTON, ASSIGNOR TO DUMOR NATIONAL CHEMICAL COMPANY, OF LACEY, WASHINGTON, A CORPORATION OF WASHINGTON

## EXPLOSIVE

No Drawing.

Application filed March 26, 1927. Serial No. 178,812.

This invention relates to improvements in explosives, having more particular reference to improvements in the explosive disclosed and claimed in United States Letters Patent, 5 No. 1,073,279, issued September 16, 1913, to James F. O'Brien, of Chicago, Ill., assignor to Dumor National Chemical Company, Seattle, Washington, and aims primarily to provide a more stable and dependable chlorate 10 explosive capable of more perfect detonation than the chlorate explosives heretofore in commercial use.

Contemplated by the present invention is the provision of a stump and rock blasting 15 chlorate explosive; which is non-hygroscopic; which will not deteriorate or chemically change with age; which is properly sensitive to assure its detonation by suitable predetermined means; which is of such stability 20 as to resist detonation from casual or unintentional influences, such as friction or shock in handling, or other influences to which an explosive is exposed in ordinary commercial use; which is not adversely affected by increase or reduction in temperature, either as 25 to power or as to safety; which may be manufactured in different grades or strengths without undesirably affecting its sensitivity or stability in either direction; which 30 may be manufactured at low cost, due both to the simplicity of the operations involved in its preparation and particularly to the low cost of the ingredients entering into its composition; all of which are important features 35 of the invention and are to be correlated in the broad aim of enhancing the efficiency of the present composition for general use.

The above and additional features, purposes and advantages, which will hereinafter 40 be more specifically treated are attained by such means as are described in the following specification and then more clearly pointed out in the claims, which are appended hereto and form part of this application.

45 To accomplish the purposes and secure the advantages hereinbefore set forth, I utilize as the ingredients of the present composition, materials which by virtue of their characteristics, are not adversely affected by increases 50 or reductions in temperature, and combine

these materials with modifying ingredients which contribute to the composition the desired sensitiveness to detonation of a predetermined sort and the desired stability and insensitiveness to other influences. 55

The materials which actual experience and extensive tests have demonstrated as most economical, efficient and practical for employment in the present composition and which have been found to give the best results are 60 as follows:—an oxidizing salt, such as sodium chlorate; a hydro-carbon, such as a nitrated derivative of toluene; a restrainer, such as sodium nitrate; an antiacid, such as calcium carbonate; and finely divided woody 65 matter, such as sawdust. The nitrated derivatives of toluene aforementioned which have been found suitable for employment in the present composition, are mononitrotoluol (orthonitrotoluol) and dinitrotoluol. In 70 some instances mononitrotoluol, per se, is used and in other instances a combination or intermixture of mononitrotoluol and dinitrotoluol, for illustration, when a rock blasting powder is required mononitrotoluol is 75 used alone, while, when a stump blasting powder is desired mononitrotoluol is combined with dinitrotoluol.

The formula for rock blasting powder which has been found to give uniformly good 80 results is as follows:—

|                         | Per cent |
|-------------------------|----------|
| Sodium chlorate         | 80       |
| Mononitrotoluol (crude) | 14       |
| Saw dust                | 6        |
| Total                   | 100      |

and the formula for stump blasting powder which has been productive of the best results is as follows:—

|                         | Per cent |
|-------------------------|----------|
| Sodium chlorate         | 29.84    |
| Sodium nitrate          | 45.86    |
| Calcium carbonate       | 3.31     |
| Mononitrotoluol (crude) | 2.62     |
| Dinitrotoluol (crude)   | 10.91    |
| Saw dust                | 7.46     |
| Total                   | 100      |

To prepare the composition, of either formula, as above set forth, the chemicals and

saw dust are heated sufficiently to drive off moisture and are then ground or pulverized. The drums of crude mononitrotoluol and dinitrotoluol, as received from the manufacturers, are not standardized products, the color and quality of each drum varying slightly, and in order to render such oils suitable for use in the present compositions, it has been found necessary to blend the contents of several drums of mononitrotoluol or several drums of dinitrotoluol in order to secure and obtain more uniform grades of the same. Further, the crude mononitrotoluol and dinitrotoluol when received are in a more or less solid state and the drums of same ordinarily contain small percentages of water, which latter is eliminated or driven off during the blending processes of said oils, which is accomplished by placing the contents of several drums of mononitrotoluol or dinitrotoluol in a suitable receptacle and subjecting the latter to sufficient heat (approximately 120° F.) to drive off the moisture and liquefy the oils. However, in this connection it may be well to note that, in order to preserve the volatile matter in the respective oils, the heat to which they are subjected during the liquefying and blending processes thereof must not be excessive. The dried and pulverized chemicals and saw dust are next placed in a suitable mixing machine and thoroughly or intimately mixed therein; and concurrently therewith the heated oil or intermixture of heated oils is slowly added thereto, as by spraying the same into the chemicals and saw dust during the intermixing of the latter, so that the particles of chemicals and saw dust are thoroughly impregnated, bound together and waterproofed by such oil. The resultant product or explosive obtained from the foregoing is a smooth plastic mass, which can be readily pressed into any required form and packed into cartridges for use as sticks. The explosive is substantially non-deliquescent and requires the action of a strong cap for its explosion, if ignited in the open it will simply burn without explosive action; and concussion, jar or shock without heat will not cause it to explode. The detonation of this explosive is positive and certain when acted upon by a strong cap, whether such explosive is confined or unconfined.

Heretofore, in explosives employing chlorates, as oxidizing salts, dinitrotoluol, per se, has ordinarily been used as the sensitizer, but, actual experience over an extended period has shown dinitrotoluol, per se, is not dependable, there being many instances where such explosives deteriorated so rapidly, due to various conditions, that they were virtually useless after being in storage for only very brief periods. It is therefore a primary feature of this invention to employ mononitrotoluol in combination with dinitrotoluol in order to

secure a more stable and dependable explosive, and actual experience has demonstrated that explosives employing such oils in combination, as a sensitizer, have the characteristic property of retaining indefinitely their plasticity, dependability and stability whatever be the length of time during which they are stored for temperatures varying from 30°, below zero, centigrade, to the highest temperatures to which they may be exposed under ordinary and practical conditions. They are moreover very insensitive to mechanical action, and their strength and power is substantially equivalent to high blasting explosives, but, having over the latter the valuable advantage of a lower cost price, smaller sensitiveness to mechanical action, and more particularly considerably greater resistance to cold, while having an increased sensitiveness to primers, and do not leave or give off noxious gases or fumes when exploded, being therefore especially adaptable and suitable for use in constricted or enclosed spaces.

Wherefore, it will be manifest and obvious to those skilled in the art upon an understanding of the foregoing, that the present application is predicated upon the disclosure of a composition of matter formed of certain specified ingredients, which, due to their respective characteristics, interact when combined to produce an essentially new composition possessing certain novel characteristics in both its static form and its explosion. However, it is to be understood, that the invention resides in the novel composition of matter having these distinctive attributes, and that it therefore is not limited to the particular ingredients herein named, or their specific proportions, as I am aware that substitutions may be made in the constituent ingredients, and variations in their proportions, without essential modification of the resulting composition. The relative proportions of the several ingredients may be varied within reasonable limits according to the special application for which the explosive is desired, as in some applications a high explosive effect is necessary, while, in other applications a rather retarded or slower effect is desirable, the former effect is obtained by increasing the percentage of chlorate in the composition, while, the latter effect is secured by decreasing the percentage of same.

Having thus fully described my invention, what I claim as new and desire to secure by Letters Patent is:—

1. An explosive containing a chlorate, liquid mononitrotoluol about three parts, and liquid dinitrotoluol about eleven parts.
2. An explosive containing a chlorate, liquid mononitrotoluol about three parts, liquid dinitrotoluol about eleven parts, and finely divided woody matter.

In testimony whereof I affix my signature.  
CHARLES H. WATERS.